

## UNITED STATES PATENT OFFICE

2,416,709

## METHOD OF TREATING TIN BEARING MATERIALS

Irving E. Muskat, Plainfield, N. J.

No Drawing. Application September 6, 1945,  
Serial No. 614,825

24 Claims. (Cl. 23—53)

1

This invention is directed to the recovery of tin from tin ores, including concentrated and unconcentrated ores, preferably from those containing 5 per cent by weight or more of tin.

This application is a continuation-in-part of my copending application Serial No. 469,373, filed December, 17, 1942.

In accordance with the present invention I have found that tin may be recovered efficiently and at relatively low cost from tin ores or concentrates by a process involving a reaction of the tin content thereof in a reduced state with an aqueous solution of an alkali metal hydroxide.

In the practice of the process herein contemplated a tin ore in a finely divided state is heated in the presence of a quantity of a reducing agent capable of reducing tin oxide to metallic tin, such as carbon, coal, lampblack, petroleum coke, carbon monoxide, natural gas, hydrogen, etc., for a time required and at a predetermined temperature to convert the tin content of the ore into a state capable of reacting with a solution of an alkali metal hydroxide. Thereafter the treated ore is subjected, under controlled conditions, to the action of an aqueous alkaline solution, preferably an aqueous solution of an alkali metal hydroxide such as sodium or potassium hydroxide. In order to achieve a satisfactory reaction of the reduced tin of the treated ore with the alkali metal hydroxide solution, the reaction should be conducted at a temperature of at least 75° C. and, preferably, of not less than 90° C. The preferred reaction temperature is at or slightly below the boiling point of the alkali metal hydroxide solution. After such treatment metallic tin may be recovered by any of several methods, as herein-after explained.

The process herein contemplated is effective for treatment of all types of tin ores containing from as little as 5 per cent and up to 60 per cent and even more of tin, including both high grade and low grade ores. In the case of the treatment of the high-tin ores such as ores containing above about 35 to 40 per cent of tin, it is desirable in some cases to add an inert material such as the spent residues from the leaching operation herein-after described to prevent coalescence of the tin during reduction to as great an extent as possible, and thereby make possible the recovery of a better product.

The process of my invention is especially adapted to the treatment of low grade tin concentrated or unconcentrated ores containing from about 15 to 35 per cent or less of tin, which have not been capable of commercial treatment prior to the present invention. Such ores often contain 5 per cent or more of iron in addition to silica, arsenic, antimony, sulphur, etc. If sulphur is present in an excessive amount, say about 2 per cent or more, it may be desirable in some

cases to roast the ore in accordance with conventional procedures prior to treatment in order to eliminate all or a portion of this material, thereby raising the fusion point of the ore and preventing build-up of the sulfate in the herein-after described leach liquors. On the other hand, ores containing small quantities of sulphur may be treated without roasting, since some quantity of sulphur is removed during the reduction treatment.

The reduction treatment of the ore may be effected by heating the ore in a pulverized state, for example, minus 100 or 200 mesh, in the presence of a carbonaceous reducing agent such as coal, charcoal, carbon, coke, carbon monoxide, natural gas, water gas, etc., in order to convert the tin content of the ore to a state in which it is capable of reacting with an aqueous solution of an alkali metal hydroxide. This treatment should be conducted at a temperature sufficiently high to permit a major part or all of the tin content of the ore to be converted to the aforesaid state; however, the temperature should not be so high that substantial fusion occurs and a molten pool of ore, slag or metallic tin or other molten material is formed. A ball mill or other suitable grinding device may be employed to grind the ore to the desired finely divided state. The ore may be ground to minus 20 or 60 mesh, but better yields of reactable tin are obtained if the ore is ball-milled to the mesh above stated.

The exact temperature which may be utilized in the reducing treatment is dependent largely upon the nature of the ore subjected to reduction. Thus, some Bolivian ores fuse or melt to a very serious extent at a temperature of about 1600° F. On the other hand, other Bolivian ores and many Mexican ores may be subjected to temperatures as high as about 1800° or 1900° F. without encountering serious fusion. Primarily the ore should be reduced at a temperature such that a material is produced in which a major portion of the tin may be converted to a water soluble stannate by reaction with an aqueous solution of an alkali metal hydroxide. The reaction is preferably carried out in the presence of an oxidizing agent capable of oxidizing metallic tin in an alkaline medium, as herein-after described. Slight amounts of fusion resulting in some sintering of the ore undergoing treatment may be tolerated in most cases. On the other hand, fusion to an extent such that pools of molten material are formed is detrimental and should be avoided. In general, satisfactory results are usually obtained within a temperature range of about 1400 or 1500 to about 2000° F. and for most tin ores a temperature of from about 1600 to 1900° F. is most effective. A preferred temperature range is from about 1650 to 1850° F.

The reducing agent used in effecting reduction

2

of the ore should be present in amounts at least sufficient to render all or most of the tin content of the ore soluble in an aqueous solution of an alkali. Both gaseous reducing agents, such as carbon monoxide, water gas, hydrogen or natural gas, and solid reducing agents may be used, as pointed out above. I have been able to secure particularly effective results by conducting the reduction of the finely ground ore in the presence of a solid carbonaceous material, preferably in powdered form and preferably of a mesh corresponding substantially to the mesh of the ore. These solid carbonaceous reducing agents are preferred because they are easier to handle and because they have the property of minimizing fusion and sintering of the ore. Solid carbonaceous materials containing both nonvolatile and volatile carbonaceous reducing agents, such as anthracite or bituminous coal, are most suitable for this purpose. Bituminous coal is preferred because of its relative cheapness and availability.

The period of time over which the ore is subjected to the reducing treatment is capable of considerable variation, being largely dependent upon the activity of the ore undergoing treatment and the temperature of treatment. Generally speaking, the time required is shorter where the temperature is high than where a lower temperature is used. In any case, however, unduly prolonged heat treatment of the ore is detrimental and should be avoided. The actual optimum time at the reduction temperature is usually quite short and usually does not exceed about 30 to 40 minutes for low-grade ores. From data obtained by carrying out experiments in a reduction furnace, it appears that low-grade ores may be reduced to a good product in a matter of from about 8 to 12 minutes and even less. These figures include the time required to heat the ore up to the reduction temperature, which in typical instances was shown to be in the order of about 3 to 5 minutes. The reduction may be effected in any suitable furnace, such as a hearth type furnace, for example, a multiple hearth, Wedge type furnace, or a rotary furnace.

The amount of reducing agent utilized is, in general, dependent upon the temperature of treatment and the type of furnace in which reduction is effected. It has been observed that fusion of the ore may be substantially decreased and minimized when the process is conducted in the presence of an excess of solid carbonaceous material such as carbon or coal. In treatment of ores, particularly low grade ores containing from about 15 to 35 per cent of tin, not less than about twice the amount of carbon or coal required to reduce tin to the metallic state and form carbon monoxide is preferred. When this reduction is conducted in a continuous manner by use of a rotary kiln or a multiple hearth furnace or other similar device, not less than about 15 to 20 per cent by weight of carbon or coal based upon the weight of the ore is used for most cases, since with these amounts of solid carbonaceous material the tendency of the ore to fuse and sinter at the temperature of reduction is greatly lessened. In general, coal in excess of about 30 per cent by weight is undesirable where the temperature is unduly high or the treatment unduly long because coking may occur. The minimum or theoretical amount of bituminous coal, for example, required for reduction of the tin in a typical low-grade Bolivian ore of about 20 per cent tin content is about 5 per cent of the weight of the ore.

Following the reducing treatment the ore may be cooled in a nonoxidizing atmosphere to prevent reoxidation of the tin. The reduced ore after this cooling treatment usually is in the form of a black or dark colored pulverulent or granular mass containing tin in dispersed small particles in a form soluble in an aqueous alkali solution. Sometimes the mass may be more or less clinkered or caked and may require pulverizing or grinding treatment, say to minus 100 or 200 mesh, prior to or in conjunction with the aqueous alkali treatment. In the preferred operation, the reduced ore prior to the aqueous alkali treatment should be in a finely divided state such as set forth above. The exact nature of the reducing reactions is not known, although it is possible that the tin is reduced to a finely divided metallic state, the particles being separated by the excess coal and by other materials in the reduced ore. In any event, the treated ore is amenable to reaction with an aqueous solution of an alkali metal hydroxide.

The ore after the reduction treatment may be subjected to any of several types of aqueous alkaline treatments. If desired, it may be treated with an aqueous solution of sodium hydroxide under conditions such that a liquid extract of sodium stannate is produced. Alternatively, it may be subjected to treatment with an aqueous solution containing at least 15 per cent of sodium hydroxide or its equivalent of another alkali metal hydroxide, and, generally, not substantially more than 1.5 times the theoretical amount of the hydroxide required to react with the tin in the reduced ore. In such a case reaction of the aqueous alkali solution with the tin in the ore occurs rapidly to form a substantially solid mass comprising sodium stannate crystals. This mass may then be extracted with water to dissolve the stannate and thereby to separate it from the gangue including iron and silicon impurities. Usually it is desirable to conduct this treatment in the presence of an oxidizing agent capable of oxidizing metallic tin in an alkaline medium, such as sodium nitrate, sodium hypochlorite, potassium nitrate, hydrogen peroxide, etc., in order to assist or speed up the rate of reaction. Generally, when the aforesaid solutions of sodium stannate are to be electrolyzed, 5 to 7 moles of alkali metal hydroxide are used per mole of oxidizing agent.

It is preferred that the treatment of the reduced ore with the alkali metal hydroxide solution be carried out in a countercurrent operation, either batch or continuous. In such operations the concentrations of the alkali metal hydroxide may vary widely, say from about 50 to 200 gms. per liter of solution. It is preferred to use some oxidizing agent such as  $\text{NaNO}_3$ , for example, with the alkali metal hydroxide in a concentration of at least about 10 gms. per liter of solution. A preferred aqueous alkaline treating solution for a countercurrent operation contains 130 gms.  $\text{NaOH}$  and 40 gms.  $\text{NaNO}_3$  per liter of solution. In general, the amount of alkaline treating solution used should be such as to provide an excess of the alkaline reagent over the theoretical requirements for the conversion of the tin to the stannate form; for example, an excess of about 50 to 300 per cent, preferably about 100 to 150 per cent. With the preferred solution containing 130 gms.  $\text{NaOH}$  and 40 gms.  $\text{NaNO}_3$  per liter of solution, one liter will effectively treat an amount of ore containing up to about 100 gms. of tin.

In order to effect a satisfactory reaction between the aqueous alkali metal hydroxide solution and the reduced ore, it is necessary to maintain a reaction temperature of at least about 75° C. and preferably above 90° C. and as high as the boiling point of the solution during a substantial period of the treatment. At temperatures below this level the reaction occurs at such a low rate that it is ineffective for use in a commercial operation. When dilute solutions are used to extract the tin, heat must be applied to establish this temperature. On the other hand, in a batch operation, when a solution containing in excess of 150 gms. of an alkali metal hydroxide per liter of solution is used, say from 200 to 350 gms. per liter, the heat evolved during the extraction of tin is sufficient to establish the required temperature condition. This is particularly true where the amount of solution is limited to approximately the stoichiometric equivalent of the tin.

The aqueous solution of sodium stannate and/or sodium stannite produced may be treated by various convenient methods to recover tin. If desired, the solution may be concentrated and the sodium stannate crystallized out of solution. This compound may be redissolved and the solution electrolyzed to produce metallic tin. Alternatively, tin oxide may be precipitated from solution and the oxide smelted to the metallic state.

The following example is illustrative of a countercurrent method of reacting and leaching reduced tin ore with an alkaline solution in accordance with the present invention. This example is of a three-stage batch-countercurrent method carried out on a pilot plant scale.

#### Example 1

The ore preparatory to the countercurrent leaching was roasted and reduced as follows:

Ore containing about 21% tin, 22% iron, 19% silica, 2% sulfur, and other impurities in minor amounts was roasted in an oil-fired rotary furnace in an oxidizing atmosphere at a temperature of about 1500° F. The roasted ore, which contained about 0.7% sulfur, was ball-milled to a particle size passing a 100-mesh screen. 100 parts by weight of the milled ore was intimately mixed with 20 parts of powdered bituminous coal. The mixture was fed into an oil-fired rotary furnace maintained at a maximum temperature of about 1800° F. and operated with a reducing atmosphere. The ore-coal mixture was fed in at a rate such that it passed through the furnace in about 15 minutes. The reduced ore was cooled in a non-oxidizing atmosphere and then ball-milled to pass a 100-mesh screen.

This finely divided reduced ore was then treated in a batch-countercurrent system as follows:

367 lbs. of reduced ore was introduced into a mixing tank together with 175 gallons of a partly spent solution containing about 104 gms. NaOH, 32 gms. NaNO<sub>3</sub> and 20 gms. Sn per liter, which was obtained from the following ore treating step. This mixture was heated at a temperature of about 105° C., the approximate boiling point of the solution, for a period of 1 hour with constant agitation. The mixture was cooled and allowed to settle for a period of about 18 hours. The solution, which now contained 56 gms. Sn per liter, was decanted and a sample of the solution was concentrated to precipitate sodium stannate, which was then redissolved and the solution electrolyzed to recover tin.

The partly spent ore, containing 7% undissolved tin, was then mixed with 150 gallons of a partly spent solution, containing about 113 gms. NaOH, 35 gms. NaNO<sub>3</sub> and 6 gms. Sn per liter, which was obtained from the following ore treating step, under the same conditions as in the first treatment. The solution decanted from this mixture, after settling, was used in treating the fresh ore as described above.

10 The nearly spent ore, containing 4% undissolved tin, was treated with 150 gallons of an aqueous solution containing 130 gms. NaOH, 40 gms. NaNO<sub>3</sub> per liter, and no tin, under the same conditions as in the preceding two steps. The spent residue from this treatment still contained 3% of insoluble tin, and the recovery of tin based on the total tin content of the original ore was about 90%.

15 It is of course manifest that the number of steps of operation of the countercurrent leaching method described in the foregoing illustrative example may be increased or decreased as desired, or may be carried out in a continuous countercurrent operation, employing conventional procedures. It is further manifest that the details as to time and temperature of reduction and proportions of coal to ore may be varied, as may also the concentration of the alkaline solution, the proportions of sodium hydroxide to sodium nitrate and the temperature of reaction of the alkaline solution with the reduced ore, all as hereinabove set forth.

20 The following examples further illustrate my invention:

#### Example 2

25 100 parts by weight of a Mexican tin ore concentrate, ground to 200 mesh and containing 27 per cent tin and 20 per cent iron, was mixed with 15 parts by weight of powdered bituminous coal and the mixture was heated for one hour at a temperature of 1700° F. by passing it through a multiple hearth roasting furnace. The reduced ore was cooled in a non-oxidizing atmosphere and then ball-milled to pass a 100-mesh screen. The treated ore was then extracted with an aqueous solution containing 10 grams per liter of sodium hydroxide and 3.22 grams per liter of sodium nitrate at a temperature of the boiling point of the solution and the extraction continued for three hours. The solution was separated from the residual ore, the ore was washed with water, and the resulting combined solutions, containing 6 grams of sodium hydroxide and 4 grams of tin per liter, were concentrated to precipitate sodium stannate. This sodium stannate was re-dissolved and the solution electrolyzed to recover metallic tin. No appreciable amount of the iron and only a minor quantity of silica were extracted with the tin in the leaching process. Attempts to leach the tin at 60° C. were unsuccessful due to the extremely slow rate at which the tin dissolved.

#### Example 3

30 35 A quantity of ore reduced and ground as in Example 2 was mixed with a solution containing 200 grams of sodium hydroxide and 142 grams of sodium nitrate per liter of solution, in the proportion of 1.1 moles of sodium hydroxide to 1 of tin in the ore. The temperature was maintained at 100 to 120° C. The reaction occurred rapidly with evolution of ammonia and heat, a stiff mud being obtained. This mass was ground as above and extracted with water, and the resulting solution was electrolyzed to recover the tin.

## Example 4

The process of Example 2 was repeated, using a solution containing 200 grams of sodium hydroxide per liter of solution and maintaining the temperature approximately at the boiling point of the solution. The resulting solution contained 92 grams of tin per liter of solution after a 4 hour leach. Only minor quantities of tin were extracted when the leaching process was conducted at 60° C.

Although the invention has especial value for the treatment of ores, including naturally occurring minerals containing tin, and ore concentrates, the invention may also be applied to the treatment of other tin oxide containing materials including chemically precipitated stannic oxide, tin oxide wastes, etc. While the invention has been described with particular reference to sodium hydroxide, other alkali metal hydroxides such as potassium or lithium hydroxide or mixtures thereof may be used if desired. It is not intended that the specific details of the illustrative embodiments of the invention shall be regarded as limitations upon the scope of the invention, except in so far as included in the accompanying claims.

I claim:

1. In the method of recovering tin from a low grade tin ore containing a substantial amount of metallic impurities including iron and at least about 5% of tin in a form in which it is in a substantially aqueous alkali-insoluble state, the steps comprising heating such ore in the presence of an excess of a solid carbonaceous reducing agent at a temperature of at least about 1400° F. but below that at which the ore fuses under conditions such that reduced ore containing tin in dispersed small particles in a form soluble in aqueous alkali solution is produced, reacting the product of such treatment containing the said soluble tin with an aqueous solution of an alkali metal hydroxide at a temperature of at least about 75° C., so as to convert the tin to a water-soluble tin compound and effect solution thereof substantially uncontaminated with iron, and separating the resulting solution from the residual ore.

2. The method set forth in claim 1 wherein the solid carbonaceous reducing agent is present in an amount of from 15 to 30%, based on the weight of the ore, said percentage varying in direct proportion to the tin content of the ore.

3. The method set forth in claim 1 wherein the solid carbonaceous reducing agent is present in an amount of from 15 to 30%, based on the weight of the ore, said percentage varying in direct proportion to the tin content of the ore, and wherein the ore contains from 15 to 35% of tin.

4. In the method of recovering tin from a low grade tin ore containing a substantial amount of metallic impurities including iron and at least about 5% of tin in a form in which it is in a substantially aqueous alkali-insoluble state, the steps comprising heating such ore in the presence of an excess of a solid carbonaceous reducing agent at a temperature of at least about 1400° F. but below that at which the ore fuses under conditions such that reduced ore containing tin in dispersed small particles in a form soluble in aqueous alkali solution is produced, reacting the product of such treatment containing the said soluble tin with an aqueous solution of an alkali metal hydroxide and an oxidizing agent capable of oxidizing metallic tin in an alkaline medium, at a temperature of at least about 75° C., so as to convert the

tin to a water-soluble tin compound and effect solution thereof substantially uncontaminated with iron, and separating the resulting solution from the residual ore.

5. The method set forth in claim 4 wherein the oxidizing agent is sodium nitrate and the alkali metal hydroxide is sodium hydroxide.

6. The method set forth in claim 4 wherein the oxidizing agent is an alkali metal nitrate.

10 7. The method set forth in claim 4 wherein the oxidizing agent is sodium hypochlorite.

8. In the method of recovering tin from a low grade tin ore containing a substantial amount of metallic impurities including iron and at least about 5% of tin in a form in which it is in a substantially aqueous alkali-insoluble state, the steps comprising heating such ore in the presence of at least about 15% by weight of a solid carbonaceous reducing agent, based on the weight of the ore, at a temperature of at least about 1400° F., but below that at which the ore fuses under conditions such that reduced ore containing tin in dispersed small particles in a form soluble in aqueous alkali solution is produced, and reacting the product of such treatment containing the said soluble tin with an aqueous solution of an alkali metal hydroxide at a temperature of at least about 75° C., so as to convert the tin to a water-soluble tin compound which may be dissolved without solution of iron in objectionable amounts.

30 9. The method of claim 8 in which the ore contains from about 15 to 35% of tin.

10. In the method of recovering tin from a low grade tin ore containing a substantial amount of metallic impurities including iron and at least about 5% of tin in a form in which it is in a substantially aqueous alkali-insoluble state, the steps comprising heating such ore in the presence of at least about 15% by weight of a solid carbonaceous reducing agent, based on the weight of the ore, at a temperature of at least about 1400° F. but below that at which the ore fuses under conditions such that reduced ore containing tin in dispersed small particles in a form soluble in aqueous alkali solution is produced, and reacting the product of such treatment containing the said soluble tin with an aqueous solution of an alkali metal hydroxide and an oxidizing agent capable of oxidizing metallic tin in an alkaline medium, at a temperature of at least about 75° C., so as to convert the tin to a water-soluble tin compound which may be dissolved without solution of iron in objectionable amounts.

11. In the method of recovering tin from a low grade tin ore containing a substantial amount of metallic impurities including iron and at least about 5% of tin in a form in which it is in a substantially aqueous alkali-insoluble state, the steps comprising heating such ore in the presence of at least about 15% by weight of a solid carbonaceous reducing agent, based on the weight of the ore, at a temperature of at least about 1400° F. but below that at which the ore fuses under conditions such that reduced ore containing tin in dispersed small particles in a form soluble in aqueous alkali solution is produced, and reacting the product of such treatment containing the said soluble tin with an aqueous solution of an alkali metal hydroxide and an alkali metal nitrate at a temperature of at least about 75° C., so as to convert the tin to a water-soluble tin compound which may be dissolved without solution of iron in objectionable amounts.

12. In the method of recovering tin from a low grade tin ore containing a substantial amount of

metallic impurities including iron and at least about 5% of tin in a form in which it is in a substantially aqueous alkali-insoluble state, the steps comprising heating such ore in the presence of at least about 15% by weight of a solid carbonaceous reducing agent, based on the weight of the ore, at a temperature of at least about 1400° F. but below that at which the ore fuses under conditions such that reduced ore containing tin in dispersed small particles in a form soluble in aqueous alkali solution is produced, and reacting the product of such treatment containing the said soluble tin with an aqueous solution of an alkali metal hydroxide and sodium hypochlorite at a temperature of at least about 75° C., so as to convert the tin to a water-soluble tin compound which may be dissolved without solution of iron in objectionable amounts.

13. In the method of recovering tin from a low grade tin ore containing a substantial amount of metallic impurities including iron and at least about 5% of tin in a form in which it is in a substantially aqueous alkali-insoluble state, the steps comprising heating such ore in the presence of at least about 15% by weight of a solid carbonaceous reducing agent, based on the weight of the ore, at a temperature of at least about 1400° F. but below that at which the ore fuses under conditions such that reduced ore containing tin in dispersed small particles in a form soluble in aqueous alkali solution is produced, and reacting the product of such treatment containing the said soluble tin with an aqueous solution of an alkali metal hydroxide and sodium hypochlorite at a temperature of at least about 75° C., so as to convert the tin to a water-soluble tin compound which may be dissolved without solution of iron in objectionable amounts.

14. In the method of recovering tin from a low grade tin ore containing a substantial amount of metallic impurities including iron and at least about 5% of tin in a form in which it is in a substantially aqueous alkali-insoluble state, the steps comprising heating such ore in the presence of a solid carbonaceous reducing agent at a temperature above about 1600° F. but below that at which the ore fuses under conditions such that reduced ore containing tin in dispersed small particles in a form soluble in aqueous alkali solution is produced, and reacting the product of such treatment containing the said soluble tin with an aqueous solution of an alkali metal hydroxide, at a temperature of at least about 75° C., so as to convert the tin to a water-soluble tin compound which may be dissolved without solution of iron in objectionable amounts.

15. In the method of recovering tin from a low grade tin ore containing a substantial amount of metallic impurities including iron and a substantial quantity of inert components and at least about 5% of tin in a form in which it is in a substantially aqueous alkali-insoluble state, the steps comprising heating such ore in a finely divided state in a reducing atmosphere at a temperature below that at which the ore fuses under conditions such that reduced ore containing tin in dispersed small particles in a form soluble in aqueous alkali solution is produced, and reacting the product of such treatment containing the said soluble tin with an aqueous solution of an alkali metal hydroxide, at a temperature of at least about 75° C., so as to convert the tin to a water-soluble tin compound which may be dissolved without solution of iron in objectionable amounts.

16. In the method of recovering tin from a low

grade tin ore containing a substantial amount of metallic impurities including iron and a substantial quantity of inert components and at least about 5% of tin in a form in which it is in a substantially aqueous alkali-insoluble state, the steps comprising heating such ore in a finely divided state in a reducing atmosphere at a temperature below that at which the ore fuses under conditions such that reduced ore containing tin in dispersed small particles in a form soluble in aqueous alkali solution is produced, reacting the product of such treatment containing the said soluble tin with an aqueous solution of an alkali metal hydroxide, at a temperature of at least about 75° C., so as to convert the tin to a water-soluble tin compound and effect solution thereof substantially uncontaminated with iron, and separating the resulting solution from the residual ore.

20 17. In the method of recovering tin from a low grade tin ore containing a substantial amount of metallic impurities including iron and at least about 5% of tin in a form in which it is in a substantially aqueous alkali-insoluble state, the steps comprising heating such ore in the presence of at least about twice the amount of solid carbonaceous reducing agent required to reduce the tin content of the ore, at a temperature of at least about 1400° F. but below that at which the ore fuses under conditions such that reduced ore containing tin in dispersed small particles in a form soluble in aqueous alkali solution is produced, reacting the product of such treatment containing the said soluble tin with an aqueous solution of an alkali metal hydroxide and an oxidizing agent capable of oxidizing metallic tin in an alkaline medium, at a temperature of at least about 75° C., so as to convert the tin to a water-soluble tin compound and effect solution thereof substantially uncontaminated with iron, and separating the resulting solution from the residual ore.

25 18. In the method of recovering tin from a low grade tin ore containing a substantial amount of metallic impurities including iron and at least about 5% of tin in a form in which it is in a substantially aqueous alkali-insoluble state, the steps comprising heating such ore in a finely divided state in the presence of an excess of a powdered carbonaceous reducing agent at a temperature of at least about 1400° F. but below that at which the ore fuses under conditions such that reduced ore containing tin in dispersed small particles in a form soluble in aqueous alkali solution is produced, cooling and pulverizing the reduced ore, reacting the product of such treatment containing the said soluble tin with an aqueous solution of an alkali metal hydroxide and an oxidizing agent capable of oxidizing metallic tin in an alkaline medium, at a temperature between about 75° C. and about the boiling point of the said solution, so as to convert the tin to a water-soluble tin compound and effect solution thereof substantially uncontaminated with iron, and separating the resulting solution from the residual ore.

30 19. In the method of recovering tin from a low grade tin ore containing a substantial amount of metallic impurities including iron and at least about 5% of tin in a form in which it is in a substantially aqueous alkali-insoluble state, the steps comprising heating such ore in a finely divided state in the presence of an excess of a powdered carbonaceous reducing agent at a temperature of at least about 1400° F. but below that

at which the ore fuses, for about 3 to about 40 minutes, under conditions such that reduced ore containing tin in dispersed small particles in a form soluble in aqueous alkali solution is produced, cooling and pulverizing the reduced ore, reacting the product of such treatment containing the said soluble tin with an aqueous solution of an alkali metal hydroxide and an oxidizing agent capable of oxidizing metallic tin in an alkaline medium, at a temperature between about 75° C. and about the boiling point of the said solution, so as to convert the tin to a water-soluble tin compound and effect solution thereof substantially uncontaminated with iron, and separating the resulting solution from the residual ore.

20. In the method of recovering tin from a low grade tin ore containing a substantial amount of metallic impurities including iron and about 5% to 35% of tin in a form in which it is in a substantially aqueous alkali-insoluble state, the steps comprising heating such ore in a finely divided state in a reducing atmosphere at a temperature of at least about 1400° F. but below that at which the ore fuses under conditions such that reduced ore containing tin in dispersed small particles in a form soluble in aqueous alkali solution is produced, and reacting the product of such treatment containing the said soluble tin with an aqueous solution of an alkali metal hydroxide, at a temperature between about 75° C. and about the boiling point of the said solution, so as to convert the tin to a water-soluble tin compound which may be dissolved without solution of iron in objectionable amounts.

21. In the method of recovering tin from a low grade tin ore containing a substantial amount of metallic impurities including iron and about 5% to 35% of tin in a form in which it is in a substantially aqueous alkali-insoluble state, the steps comprising heating such ore in a finely divided state in a reducing atmosphere at a temperature of at least about 1400° F. but below that at which the ore fuses under conditions such that reduced ore containing tin in dispersed small particles in a form soluble in aqueous alkali solution is produced, and reacting the product of such treatment containing the said soluble tin with an aqueous solution of an alkali metal hydroxide and an oxidizing agent capable of oxidizing metallic tin in an alkaline medium, at a temperature between about 75° C. and about the boiling point of the said solution, so as to convert the tin to a water-soluble tin compound which may be dissolved without solution of iron in objectionable amounts.

22. In the method of recovering tin from a low grade tin ore containing a substantial amount of metallic impurities including iron and about 5% to 35% of tin in a form in which it is in a substantially aqueous alkali-insoluble state, the steps comprising heating such ore in a finely divided state in a reducing atmosphere at a temperature of at least about 1400° F. but below that at which the ore fuses under conditions such that reduced ore containing tin in dispersed small particles in a form soluble in aqueous alkali solution is produced, cooling and pulverizing the reduced ore and reacting the product of such treatment containing the said soluble tin with an aqueous solution of an alkali metal hydroxide and an oxidizing agent capable of oxidizing metallic tin in an alkaline medium, at a temperature between about 75° C. and about the boiling point of the said solution, so as to convert the tin to a water-

soluble tin compound which may be dissolved without solution of iron in objectionable amounts.

23. In the method of recovering tin from a low grade tin ore containing a substantial amount of metallic impurities including iron and at least about 5% of tin in a form in which it is in a substantially aqueous alkali-insoluble state, the steps comprising heating such ore in a finely divided state in the presence of a powdered carbonaceous reducing agent at a temperature of at least about 1400° F. but below that at which the ore fuses under conditions such that reduced ore containing tin in dispersed small particles in a form soluble in aqueous alkali solution is produced, and reacting the product of such treatment containing the said soluble tin with an aqueous solution of an alkali metal hydroxide and an oxidizing agent capable of oxidizing metallic tin in an alkaline medium, at a temperature of about the boiling point of the said solution, so as to convert the tin to a water-soluble tin compound which may be dissolved without solution of iron in objectionable amounts.

24. In the method of recovering tin from a low grade tin ore containing a substantial amount of metallic impurities including iron and at least about 5% of tin in a form in which it is in a substantially aqueous alkali-insoluble state, the steps comprising heating such ore in a finely divided state in the presence of a powdered carbonaceous reducing agent at a temperature of at least about 1400° F. but below that at which the ore fuses under conditions such that reduced ore containing tin in dispersed small particles in a form soluble in aqueous alkali solution is produced, and reacting the product of such treatment containing the said soluble tin with an aqueous solution of an alkali metal hydroxide and an oxidizing agent capable of oxidizing metallic tin in an alkaline medium, at a temperature between about 75° C. and about the boiling point of the said solution, so as to convert the tin to a water-soluble tin compound which may be dissolved without solution of iron in objectionable amounts.

IRVING E. MUSKAT.

#### REFERENCES CITED

The following references are of record in the prior application 469,373 referred to in this patent:

#### UNITED STATES PATENTS

| Number       | Name          | Date           |
|--------------|---------------|----------------|
| 55 1,902,735 | Tamaru et al. | Mar. 21, 1933  |
| 883,589      | Thirot        | Mar. 31, 1908  |
| 1,018,734    | Weber         | Feb. 27, 1912  |
| 1,511,590    | Buttfield     | Oct. 14, 1924  |
| 40 859,566   | Leitch        | July 9, 1907   |
| 1,670,307    | Little        | May 22, 1928   |
| 2,055,732    | Schertel      | Sept. 29, 1936 |

#### FOREIGN PATENTS

| Number   | Country | Date          |
|----------|---------|---------------|
| 65 9,821 | British | June 14, 1889 |
| 10,309   | British | May 2, 1906   |
| 984      | British | A. D. 1853    |
| 614      | British | A. D. 1915    |

#### OTHER REFERENCES

Tin, by C. L. Mantell, The Chemical Catalog Co., N. Y., 1929, pp. 123, 124, 130, 133, 138, 143, 144, 265, 339, 340. (Copy in Div. 3.)